

# UNITED STATES PATENT OFFICE.

FREDERICK A. ABEL, OF LONDON, AND JAMES DEWAR, OF CAMBRIDGE,  
ENGLAND.

## GELATINOUS EXPLOSIVE.

SPECIFICATION forming part of Letters Patent No. 425,648, dated April 15, 1890.

Application filed August 27, 1889. Serial No. 322,121. (No specimens.) Patented in England May 27, 1889, No. 8,718; in France August 19, 1889, No. 198,946; in Belgium August 21, 1889, No. 87,455, and in South Australia September 24, 1889, No. 1,418.

*To all whom it may concern:*

Be it known that we, FREDERICK AUGUSTUS ABEL, knight, and JAMES DEWAR, professor of chemistry, citizens of England, residing, respectively, at 1 Adam Street, Adelphi, in London, in the county of Middlesex, England, and at 1 Scoop Terrace, Cambridge, in the county of Cambridge, England, have invented a new and useful Improvement in the Manufacture of Explosives, (for which we have obtained Letters Patent in South Australia, dated September 24, 1889, No. 1,418; in France, by Certificate of Addition, dated August 19, 1889, No. 198,946; in Belgium, by Certificate of Addition, dated August 21, 1889, No. 87,455, and in Great Britain, by an application for patent, which patent when granted will bear date May 27, 1889, No. 8,718,) of which the following is a specification.

20 The gelatinous explosives produced by combinations of nitro-cellulose and nitro-glycerine, with or without other ingredients, exert great disruptive force when they explode, and are therefore not suited for ammunition purposes.

Our invention relates to an improvement in the manufacture of such explosives whereby we moderate the force and rapidity of their explosion, giving it a propulsive instead of a 30 disruptive character, so that they are adapted for ammunition purposes, the permanency of the compound without change being at the same time secured. For this purpose we combine tannin with the nitro-cellulose or 35 nitro-glycerine or with both in either of two ways. We either dissolve the nitro-cellulose—such as gun-cotton or pyroxyline—by any of the known solvents—such as acetone or acetic ether—and we add the tannin ingredient to the solution; or we first dissolve the tannin ingredient in the acetone or its analogue and use this solution as the medium

of incorporation with the nitro-glycerine. We thus produce a compound which, when the solvent is eliminated by extraction with 45 water or by evaporation, or both, is a tough hard substance that can be granulated or otherwise treated for use as an explosive.

Instead of employing nitro-cellulose alone in forming the compound, as above described, 50 we employ with it various proportions of nitro-glycerine, and we thus obtain a compound of soluble nitro-cellulose or of gun-cotton (insoluble nitro-cellulose) with nitro-glycerine and tannin in a gelatinous condition, 55 which may be rolled into sheets, drawn into wire, or otherwise treated for use as an explosive.

With the compounds produced as above described may be incorporated various proportions of oxidizing agents—such as nitrates of potassium, sodium, ammonium, and barium—and oxidizable substances—such as lamp-black or graphite—and hydrocarbons—such as paraffine, vaseline, and naphthaline, 65 cellulose, fatty oils, and fats or nitro-derivatives of hydrocarbons.

The proportion of tannin added for the purposes of our invention may be varied. In treating gun-cotton alone we have found the 70 proportion of ninety parts of gun-cotton and ten parts of tannin to give good results.

In the case of a compound of gun-cotton and nitro-glycerine we have employed the following proportions with advantage: 75

|                           | Per cent. | Per cent. | Per cent. |
|---------------------------|-----------|-----------|-----------|
| Nitro-glycerine . . . . . | 55        | 35        | 40        |
| Gun-cotton . . . . .      | 35        | 55        | 40        |
| Tannin . . . . .          | 10        | 10        | 20        |

Under the term "tannin" is to be understood any of the substances that are sold commercially under the name of "tannic acid." We prefer, however, to use gallotannic acid for the purpose of our invention. 80

Having thus described the nature of our invention and the best means we know of carrying the same into practical effect, we claim—

- 5 As a new article of manufacture, a gelatinous explosive consisting of nitro-glycerine and nitro-cellulose to which tannin is added, whereby the explosive is rendered of a propulsive instead of a disruptive character, substantially as described.

In testimony whereof we have signed our names to this specification, in the presence of

two subscribing witnesses, this 9th day of August, A. D. 1889.

F. A. ABEL.  
J. DEWAR.

Witnesses:

OLIVER IMRAY,  
U. S. Patent Agent, 28 Southampton Buildings, London, W. C.

JNO. P. M. MILLARD,  
Clerk to Messrs. Abel & Imray, Consulting Engineers and Patent Agents, 28 Southampton Buildings, London W. C.